

May 10, 1932.

A. L. CLAPP

1,857,497

METHOD OF SURFACE FINISHING PAPER OR FIBER BOARD AND PRODUCT OF SAME

Filed Feb. 14. 1927



Fig. 1



Fig. 4



Fig. 2

Inventor:  
Albert L. Clapp.  
by  
Cahier Brown Greenberg Hall  
Atty.

## UNITED STATES PATENT OFFICE

ALBERT L. CLAPP, OF DANVERS, MASSACHUSETTS

## METHOD OF SURFACE FINISHING PAPER OR FIBER BOARD AND PRODUCT OF SAME

Application filed February 14, 1927. Serial No. 168,224.

This invention relates to the surface finishing of paper, and more particularly relatively thick papers such as fiberboard, while in the course of manufacture on modern 5 papermaking machines and has for its object the production of a product having a high finish or glaze and adapted for use as trunk-board, suitcase-board, or for use in other capacities where a highly finished product is 10 desired.

In accordance with the method of the present invention, a board is formed on one of the usual types of papermaking machines, passed over driers, and then immediately before 15 or during calendering, an aqueous solution of a glaze-imparting sizing, such as sodium silicate solution, is applied on either or both faces of the board. Such sizing material penetrates rapidly into the surface portion of 20 the board, but inasmuch as the board immediately passes into the nip of the calender, there is an insufficient time interval to produce a complete penetration of the solution through the board, and accordingly a crushing or tearing of the board while under heavy 25 pressure in the nip of the rolls is prevented. As the surface-impregnated board passes through the rolls, which are preferably maintained hot, the fuzz on its surface is ironed 30 down and pressed into the silicate, which retains it in such condition and hardens or sets on drying to impart a high finish or glaze to the board.

It is essential that the board being finished 35 by my method be either unsized or filled with material having high affinity for sodium silicate solution. For instance if it be attempted so to finish a sized board, it is found that the calender rolls are gummed and the board 40 tends to stick to and wind around the rolls, as a sized board so resists the penetration of the silicate solution that a considerable portion of the solution is retained on the rolls. When, on the other hand, the board is unsized 45 or filled with material having high affinity for silicate solution, the solution penetrates rapidly into its surface portion, so that but little remains on the rolls and accordingly practically no difficulty is encountered during 50 calendering.

The applicability of the present invention may best be understood by reference to a specific example of procedure which is to be described in conjunction with the accompanying drawings, wherein

55

Figure 1 represents in side elevation a portion of the dryers and a stack of calender rolls, certain of which rolls receive the silicate solution from receptacles and apply it to the faces of the board.

60

Figure 2 represents in plan view the calender stack.

Figure 3 is a section through the two upper calender rolls, on the line 3—3 of Figure 2.

Figure 4 shows an enlarged section through a board surface-finished as herein described.

65

Referring to the drawings, the board S is passed from the dryer rolls 7 of the machine under a guide and tension roll 8 to the top of the calender stack and then successively 70 between each of the pairs of superposed rolls to the bottom of the stack, whereupon, if desired, it may be slit and reeled. As shown, the sizing is applied to the sides of each of the uppermost calender rolls 9, 9a, from receptacles 10. The receptacles are constructed and arranged similarly to the water boxes, so called, sometimes employed in water-finishing paper. Each receptacle, as illustrated, 75 is provided with a bottom 10a and ends 10b, which conform accurately to the contour of the roll, so that a supply of the sizing may be maintained in the receptacle, which may be supported at its ends by brackets 11 secured to the framework 12. While rotating, each of the rolls 9, 9a picks up a film 80 of the sizing and applies it to the surface of the board with which it contacts, the thickness of the film being determined by the clearance between the roll and a doctor 13 85 extending from end to end across the receptacle 10a near its top. Of course, other methods of applying the sizing to the faces of the board immediately before or during calendering may be practised. For instance, the receptacles 10 may be arranged to apply the sizing directly to the faces of the board while 90 on the calender rolls. Or suitable coating or spraying devices may be used to apply the sizing to the faces of the board immediately 95 100

before it reaches the calender rolls or while on the rolls. As the surface-sized board passes through the calender rolls, the fuzz or nap on its surfaces is ironed down and 6 pressed into the sizing, which retains it thus and hardens or sets upon drying to produce a finished and glazed surface *a*, as shown in Figure 4.

In preparing a strong board suitable for 10 use in the manufacture of trunks and suitcases, for example, the following procedure may be adopted. Eighty parts of kraft and 20 parts of rag fiber are charged into the beater engine together with sufficient water 15 to ensure circulation of the fiber. If desired, other strong fiber, such as manila or jute, may be used in lieu of the kraft fiber. The fiber is beaten, say, for six to eight hours, so as to effect sufficient hydration of the fiber to 20 felt properly on the paper machine. The fiber is then diluted to the desired consistency and run off on a paper machine into board of the desired thickness. It is preferable, however, that the board or paper be of greater 25 than 5-point thickness, since if of insufficient thickness it becomes penetrated throughout, rather than only surface-penetrated, and is likely to become crushed or torn between the calender rolls. The furnish from which 30 the board is made may of course be varied, depending upon the quality of product which it is desired to realize. For instance, if it is desired to produce a relatively inexpensive board, a furnish composed of, say, 75% 35 ground-wood or waste papers and 25% sulphite fiber and beaten for about one hour before running off on a paper machine, may be employed. Or, if it is desired to produce a white board, the furnish may be composed 40 of bleached sulphite or rag fiber, either alone or in admixture. In any of the furnishes hereinbefore given, 20% to 50% leather scrap may be used in lieu of cellulosic fiber. The 45 leather scrap, when thoroughly beaten out, say for five to six hours, may be advantageous, as it enhances the felting power of the furnish and apparently increases the wet strength of the board, so that such board while wet on the machine need be handled 50 with less care. After the board is felted, it is passed over the usual driers, and thence through the calender rolls. In passing 55 through the calenders, sodium silicate solution is applied to its surfaces from the receptacles 10. The solution is preferably about 20° Baumé, as this produces adequate penetration into the board, and the desired finish. If a very dilute or very concentrated solution were employed, difficulty would be encountered, as a dilute solution would not impart 60 of the desired body and finish to the board, whereas a concentrated solution would not penetrate into the board with sufficient rapidity so that the calender rolls would likely 65 become gummed and the board tend to

stick and wind up on the rolls. If desired, pigments such as ochre, lampblack, or the like may be added to the silicate solution to produce a coloring of the surface of the board. Preferably, also, the calenders are maintained hot, say at 160° to 180° F., as a better 70 finish is produced.

In lieu of silicate solution, aqueous solutions of other glaze-imparting, water-soluble sizes, such as glue, casein, or starches converted or made soluble by alkali, may be used at the proper consistency, but silicate solution has been found to impart the best finish and at the same time the necessary body to 75 the board.

A board finished as herein described may be varnished or lacquered, or similarly surfaced with a small amount of surfacing material, in consequence of the elimination of fuzz or nap, and in consequence of the surface resistivity of the board to penetration by varnishes or lacquers containing linseed oil or similar organic solvent as the liquid vehicle. 80

A singular advantage of the method of the present invention is that a glaze or finish 85 equivalent or superior to the glaze or finish produced by calendering or supercalendering board formed of fiber and beaten for 12 to 16 hours or longer, is economically produced, for the method is carried out while the board 90 is in the course of its manufacture and without the use of special machinery.

The method herein described cannot be practised in connection with the method of tub-sizing paper, for if paper were tub-sized 100 while in the course of its manufacture it would be crushed or torn when subjected to the heavy pressure of calender rolls, particularly with modern high-speed paper machinery. When paper is tub-sized, it is customary 105 to dry the paper slowly, as by festooning it or passing it through a drying chamber, as it is of insufficient strength to pass rapidly over driers. If tub-sized paper were then calendered, the fuzz would not be ironed out 110 to produce a smooth, glazed surface such as herein described, and the hardened size would be crushed under the calender rolls. It is thus necessary, in the practice of the present invention, to apply the sizing to the 115 board immediately before passage into the nip of the calender rolls, so that only surface impregnation occurs, as the board is subjected to heavy pressure before complete penetration has been effected. Preferably, the first 120 impregnation occurs after passage through the first nip, as the tension on the paper is considerably reduced and there is hence less likelihood of tearing it.

Where sodium silicate or the other water-soluble sizes mentioned are employed, the finish is not permanent if the board is subjected to water or moisture, unless it is varnished, lacquered, or otherwise waterproofed. In accordance with my process, however, I may 125 130

produce a finish which is waterproof without the necessity of a waterproof coating. This is accomplished by incorporating into the furnish a filler capable of reacting with sodium silicate to produce a waterproofing material. For instance, if asbestos or lime, either alone or in admixture, is incorporated in proper amount into the furnish, and the furnish then formed into board and such board is treated with sodium silicate, the sodium silicate reacts with such filling material to produce a cementitious material which upon drying sets to a hard, waterproofing compound. In accordance with the process described in my application, Serial No. 94,329, filed March 12, 1926, the board is saturated with silicate solution to produce a product which is permeated throughout with the waterproofing compound. In accordance with the present process, however, the filled board is treated at the calender rolls at its surface portions only, to produce a board impregnated at its surface portion only with the waterproofing compound. If the paper were saturated with silicate solution as described in said application, and then calendered, the board would be crushed or torn. In producing a water-resistant board according to the present invention, the procedure may be as follows. To the furnish in the beater engine is added 10% to 50% asbestos, or 5% to 20% lime, or a mixture of both asbestos and lime in the desired proportion. The lime is preferably hydrated finishing lime, so called, and is added before or during the initial stages of beating, so as to be uniformly disseminated through the furnish. The asbestos fiber may be used in the form of the relatively short and inexpensive fiber, such as is commonly used in making asbestos mill-board. The asbestos fiber is preferably added after or during the latter stages of beating, so that the length of fiber may be preserved. If desired, the so-called asbestos "floats," or dust, which is inexpensive, may be used in lieu of fiber.

The filled board is treated at the calender stack with sodium silicate, which reacts at its surface portions to produce a cementitious material which functions to retain the fuzz ironed down, and upon drying sets to impart a glazed and water-resistant surface to the board.

The method of the present invention may be applied expediently in surface finishing multi-ply or liner boards in which the inner plies are formed of fiber sized as usual in the beater, and one or both outer plies are unsized or filled with asbestos, lime or the like, capable of reacting to produce a glaze-imparting waterproofing compound. After drying, the multi-ply paper is treated at the calender stack with sodium silicate, which produces the desired finish.

I do not herein claim the subject matter

of my application, Serial No. 89,502, filed February 19, 1926, wherein paper is surface-finished or glazed while in the course of its manufacture, by treating it at the calender rolls with an aqueous dispersion of wax, and more particularly a sodium silicate dispersion of such waxes. In such case, the waxes effect a surface sizing of the paper, as the sodium silicate solution is so dilute that it has practically no effect. In the present method, a water-soluble, glaze-imparting sizing is employed to effect the surface finishing and surface sizing of the paper.

Having thus described this invention, it is evident that it is capable of change and modification without departing from its spirit or scope as defined by the appended claims.

What I claim is:

1. A process of treating unsized paper after drying while in the course of its manufacture, which comprises applying an aqueous solution of a glaze-imparting sizing to the surface of the paper, and immediately calendering the same.

2. A process of treating unsized paper after drying while in the course of its manufacture, which comprises applying an aqueous solution of a glaze-imparting sizing to the surface of the paper, and immediately hot-calendering the same.

3. A process of treating unsized paper after drying while in the course of its manufacture, which comprises applying an aqueous sodium silicate solution of about 20° Baumé to the surface of the paper, and immediately calendering the same.

4. A process of treating dry, unsized paper above 5-points thickness, which comprises applying an aqueous sodium silicate solution to the surface of the paper, and immediately calendering the same.

5. A process of treating dry unsized paper above 5-points thickness, which comprises applying an aqueous sodium silicate solution containing pigments to the surface of the paper, and immediately calendering the same.

6. A process of treating dry paper filled with lime and asbestos, which comprises surface-treating the paper with an aqueous sodium silicate solution and immediately calendering the same.

7. A process of treating dry paper filled with a material capable of reacting with silicate solution to form a glaze-imparting waterproofing compound, which comprises surface-treating the paper with an aqueous sodium silicate solution, and immediately calendering the same.

8. A calendered paper sized only at its surface portion with sodium silicate, said paper having the characteristics of said sodium silicate having been applied in the form of an aqueous solution to the surface of the paper immediately before calendering.

9. A calendered paper surface-colored and surface-sized with sodium silicate, said paper having the characteristics of said sodium silicate having been applied in the form of an aqueous solution to the surface of the paper immediately before calendering.
10. A calendered paper filled with material capable of reacting with sodium silicate solution to form a waterproofing, glaze-imparting compound, and sized only at its surface portion with the reaction product of sodium silicate and the material, said paper having the characteristics of said sodium silicate solution having been applied to the surface of the paper immediately before calendering.
11. A calendered paper filled with lime and sized only at its surface portion with the reaction product of sodium silicate solution and lime, said paper having the characteristics of said sodium silicate solution having been applied to the surface of the paper immediately before calendering.
12. A calendered paper filled with lime and asbestos, sized only at its surface portion with the reaction product of sodium silicate solution and with lime and asbestos, said paper having the characteristics of said sodium silicate solution having been applied to the surface of the paper immediately before calendering.

In testimony whereof I have affixed my signature.

ALBERT L. CLAPP.

35

40

45

50

55

60